

## UNITED STATES PATENT OFFICE

WILLOUGHBY STATHAM SMITH, OF NEWTON POPPLEFORD, HENRY JOSEPH GARNETT,  
OF SEVENOAKS, AND WALTER FREDERICK RANDALL, OF EWELL, ENGLAND

## MAGNETIC ALLOY

No Drawing. Application filed February 8, 1932, Serial No. 590,777, and in Great Britain February 5, 1931.

This invention relates to improvements in magnetic alloys comprising nickel and iron and another element to increase the specific resistance.

5 The main object of this invention is the provision of magnetic alloys having a nearly constant permeability in fields of up to 1 gauss, low hysteresis loss and high specific resistance.

19 According to the present invention the alloy comprises

|        | Per cent |
|--------|----------|
| Nickel | 62-75    |
| Iron   | 10-22    |

15 and from 10-20% of an element to increase the specific resistance. As the resistance element any one or more of the following elements may be selected:—chromium, molybdenum, tungsten, vanadium, zirconium, titanium.

20 Amounts of up to about 1% of manganese, reckoned on the final alloy, may be added to promote forgeability.

25 Copper may also be added to the alloys of this invention since its presence tends to stabilize the magnetic properties, rendering them less susceptible to variations in the heat-treatment and rates of cooling. About 5% of copper may conveniently be added and when copper is present, the maximum nickel and iron contents are reduced to 72% and 20%, respectively.

35 The alloys should be substantially free from carbon, and should be prepared by melting together the purest commercial grades of the constituent ingredients, e. g. Swedish charcoal iron, Mond nickel, chromium as sold under the registered trade mark "Thermit" and electrolytic copper under such conditions, that contamination is avoided e. g. in an electric induction furnace.

40 Alloys in accordance with the invention have an almost constant permeability and very low hysteresis losses in magnetic fields ranging from zero up to about 1 gauss, and a high specific resistance. The initial permeability may be varied from quite low values up to about 400 by varying the nature 45 of the resistance increasing element and the

proportion thereof in the alloy, while the specific resistance is high for all the compositions.

In order to develop these desired magnetic properties, the alloys should be subjected to 55 a heat treatment consisting in heating them at 1100° C. for 10 minutes, followed by rapid cooling. The heat treatment should preferably be carried out in a non-oxidizing atmosphere. 60

## Example 1

## An alloy comprising:

|          | Per cent |
|----------|----------|
| Nickel   | 69.0     |
| Iron     | 16.0     |
| Chromium | 15.0     |

when forged, drawn to fine wire, annealed at 1100° C. and tested in coil form, yielded the following results:—

|           |     |     |     |     |     |     |
|-----------|-----|-----|-----|-----|-----|-----|
| H=0.1     | 3   | 5   | 7   | 1.0 | 1.5 | 2.0 |
| $\mu=103$ | 132 | 147 | 157 | 156 | 142 | 123 |

The specific resistance was 115 microhms per  $\text{cm}^3$ .

## Example 2

## An alloy comprising:—

|           | Per cent |
|-----------|----------|
| Nickel    | 67.0     |
| Iron      | 15.0     |
| Copper    | 5.0      |
| Chromium  | 12.5     |
| Manganese | 0.5      |

85 was cast to form an ingot 1 inch in diameter. This was forged to produce a rod  $\frac{1}{4}$  inch in diameter which was reduced to wire 0.04 inches in diameter by the ordinary methods and processes commonly used in wiredrawing operations. This fine wire was made up into a coil  $2\frac{1}{2}$  inches in diameter, heat treated at 1100° C. for 10 minutes, followed by rapid cooling, and tested. The following results 90 were obtained:—

|          |     |     |     |           |
|----------|-----|-----|-----|-----------|
| H=0.1    | 0.2 | 0.3 | 0.4 | 0.8 gauss |
| $\mu=65$ | 72  | 74  | 84  | 76        |

95 The specific resistance was 109 microhms per  $\text{cm}^3$ .

*Example 3*

An alloy comprising:—

|            | Per cent |
|------------|----------|
| 5 Chromium | 11.5     |
| Iron       | 18.0     |
| Copper     | 5.0      |
| Manganese  | 0.5      |

10 and nickel the remainder, when forged, drawn to fine wire, annealed at 1100° C. and tested in coil form, yielded the following results:—

15  $\mu$  had the constant value of 180 from  $H=0$  to  $H=0.03$ .

|    | H    | $\mu$ |
|----|------|-------|
| 20 | 0.07 | 210   |
|    | 0.1  | 218   |
|    | 0.2  | 191   |

The specific resistance was 112 microhms per  $\text{cm}^3$ .

*Example 4*

An alloy comprising:—

|           | Per cent |
|-----------|----------|
| Chromium  | 12.0     |
| Iron      | 20.0     |
| 30 Copper | 5.0      |
| Manganese | 0.5      |

and nickel the remainder, when forged, drawn to fine wire, annealed at 1100° C. and tested in coil form, yielded the following results:—

35  $\mu$  had the constant value of 390 from  $H=0$  to  $H=0.07$ .

|    | H   | $\mu$ |
|----|-----|-------|
| 40 | 0.1 | 540   |
|    | 0.4 | 600   |

45 The specific resistance was 115 microhms per  $\text{cm}^3$ .

*Example 5*

An alloy comprising:—

|               | Per cent |
|---------------|----------|
| 50 Molybdenum | 10.0     |
| Iron          | 15.0     |
| Copper        | 5.0      |
| Manganese     | 0.5      |

55 and nickel the remainder, when forged, drawn to fine wire, annealed at 1000° C. and tested in coil form, yielded the following results:—

|    | H    | $\mu$ |
|----|------|-------|
| 60 | 0.02 | 490   |
|    | 0.05 | 498   |
|    | 0.1  | 550   |
|    | 0.2  | 1600  |

The same alloy when annealed at 1100° C. yielded the following results:—

| H    | $\mu$ |
|------|-------|
| 0.05 | 860   |
| 0.10 | 980   |
| 0.20 | 1300  |

70 The specific resistance was 90 microhms per  $\text{cm}^3$ .

75 The corresponding titanium and vanadium alloys are not forgeable, and could only be tested as powders. In this condition, the magnetic permeability is constant up to at least 1 gauss and has a value of 70-80.

80

*Example 6*

An alloy suitable for dust cores comprises Ni 65%, Fe 15%, tungsten 20%.

Owing to their constant permeability, low 85 hysteresis losses and high specific resistance, the alloys of this invention are particularly suitable for the manufacture of the cores of coils for lump-loading telephone circuits and can also be used for the continuous loading of 90 electric conductors.

What we claim is:—

1. Magnetic substantially carbon free 95 nickel iron alloys, comprising nickel 62-75%, iron 10-22%, and 10-20% of a third element selected from the group comprising chromium, molybdenum, tungsten, vanadium, zirconium, titanium.

2. Magnetic substantially carbon free 100 nickel iron alloys comprising nickel 62-72%, iron not more than 20%, 10-20% of an element selected to increase the resistivity and about 5% of copper.

3. Magnetic substantially carbon free 105 alloys comprising nickel about 69%, iron about 16% and about 15% of an element selected to increase the resistivity.

4. Magnetic alloys as claimed in claim 2, with the addition of about 1% of manganese to promote forgeability.

5. Magnetic substantially carbon free 110 nickel iron alloys comprising nickel 62-72%, iron not more than 20%, 10-20% of an element from the group comprising chromium, molybdenum, tungsten, vanadium, zirconium and titanium, and about 5% copper.

6. Magnetic substantially carbon free 115 alloys comprising nickel about 69%, iron about 16% and about 15% of chromium.

7. Magnetic substantially carbon free 120 nickel iron alloys comprising nickel 62-75%, iron 10-22% and 11-20% of a third element selected from the group comprising chromium, molybdenum, tungsten, vanadium, zirconium, titanium, which alloys have been subjected to a heat treatment and at a temperature and for a period sufficient to anneal the alloy completely followed by rapid cooling whereby they develop an initial magnetic permeability below 500 and which does not 125 130

vary more than 20% in fields up to 0.1 gauss.

8. Magnetic substantially carbon free nickel iron alloys comprising nickel 62-75%, iron not more than 22%, and not less than 5 11% nor more than 20% of a third element selected from the group comprising chromium, molybdenum, tungsten, vanadium, zirconium and titanium.

In testimony that we claim the foregoing 10 as our invention we have signed our names this 21st day of January, 1932.

WILLOUGHBY STATHAM SMITH.

HENRY JOSEPH GARNETT.

WALTER FREDERICK RANDALL.

15

20

25

30

35

40

45

50

55

60